

## UNITED STATES PATENT OFFICE.

ARMAN E. BECKER, OF NEWARK, NEW JERSEY, ASSIGNOR TO STANDARD DEVELOPMENT COMPANY, A CORPORATION OF DELAWARE.

## ART OF PREPARING LUBRICANT-CARRIER MATERIAL.

No Drawing.

Application filed May 16, 1922. Serial No. 561,532.

To all whom it may concern:

Be it known that I, ARMAN E. BECKER, a citizen of the United States, residing at Newark, in the county of Essex and State 5 of New Jersey, have invented new and useful Improvements in the Art of Preparing Lubricant-Carrier Material, of which the following is a specification.

The present invention relates to improvements in the art of preparing lubricant-carriers and particularly the preparation of lubricant holding and distributing material of metallic character. The invention will 10 be fully understood from the following description.

In lubrication it is important that an adequate film of the lubricating agent be maintained between the surfaces concerned, and while the film holding and spreading 15 capability of surfaces varies with the lubricant used, it especially varies with the character of the metallic surface. In the case also of surfaces not directly a part of the bearing but functioning to distribute the 20 lubricant to a journal or bearing element, notably in the case of divided or fibrillar metals, so-called metal wool, this becomes 25 of importance in the realization of an increased capillary feed capacity. I have now 30 discovered that the aforesaid property of metallic surfaces can be increased by an improved treatment, applicable both to bearing and feed elements.

In practicing my invention, any material 35 amenable may be treated, and in any desired or practicable form, whether in larger units and surfaces or finely divided or the so-called wool, such as steel wool, copper wool, brass wool, Monel wool, etc., but by way 40 of an illustrative example, reference may be made to the treatment of metallic wool for use in the journal boxes of railway car trucks etc. Steel wool of suitable grade is subjected to a bath of oil, such for instance as a cylinder stock or pressure still 45 tar or any oil which in a refined or unrefined state contains small quantities of sulfur and is heated to a temperature sufficient to promote sulfurization of the metal 50 surface and preferably to about 300° F. to 500° F. The steel wool appears to have some sort of affinity for the oil at elevated tem-

peratures and particularly in the presence of sulfur soon blackens and after removal from the treating bath is found to exhibit 55 greater capacity for holding a lubricant. Instead of using the oils mentioned, there can be used heavy distillates off of pressure still tar, or distillates from Mexican petroleum or the like. For instance, a 60 Mexican water white distillate with a sulfur content 0.933% has shown advantageous results. While not to be taken as a rule I have generally found it true that those oils which carry a loosely-bound sulfur content 65 are the most useful. Where sulfur is desired in an oil not naturally containing it, sulfur can be added in the free state or other reactive form. In the presence of the sulfur the metallic surface acquires a sulfid 70 film. Without going further into the theoretical aspects of the matter, since the phenomenon is complex and not at this time entirely clear, I content myself here rather with stating the facts observed. In place 75 of immersing the metal wool in oil, it can be subjected to the proper oil vapors at the suitable temperature, and in the claims hereinafter, it will be understood that the term "oil" includes either the liquid or 80 vapor phase. It is generally preferable from the standpoint of convenience, and more satisfactory however to use the liquid.

Ordinarily mineral oils are preferable, but in some cases oily materials of vegetable 85 or animal origin may be used.

While I have described my invention by reference to certain specific examples, it will be understood that these are illustrative and not limitative, nor is the invention to be 90 considered as dependent upon the accuracy of any theories mentioned. On the contrary, it is to be regarded as limited only by the following claims, in which it is my intention to claim all inherent novelty as 95 broadly as the prior art permits.

What I claim is:

1. The process of preparing a metallic lubricant-carrier which comprises subjecting the surface of the metal to an oil with an available sulfur-content, heated to 300°- 100 500° F.

2. The process of preparing a metallic wool lubricant-carrier, which comprises

treating the metallic wool with an oil in the presence of available sulfur at a temperature of 300°-500° F.

pared by subjecting the wool to an oil in the presence of available sulfur at a temperature of 300°-500° F.

3. The process of preparing a metallic wool lubricant-carrier, which comprises treating steel wool with a petroleum oil having a loosely-bound sulfur content heated to 300°-500° F.

4. A metallic wool lubricant-carrier pre-

5. The process of preparing a metallic lubricant-carrier, which comprises forming a coating on the surface of the metallic carrier by heating said carrier in the presence of a sulfur-containing oil.

ARMAN E. BECKER.